

# UNITED STATES PATENT OFFICE.

EDWARD HOIT NUTTER, OF SAN FRANCISCO, CALIFORNIA, ASSIGNOR TO MINERALS SEPARATION AMERICAN SYNDICATE (1913) LIMITED, OF LONDON, ENGLAND.

## CONCENTRATION OF ORE.

1,170,665.

Specification of Letters Patent.

Patented Feb. 8, 1916.

No Drawing.

Application filed August 31, 1915. Serial No. 48,169.

*To all whom it may concern:*

Be it known that I, EDWARD HOIT NUTTER, a citizen of the United States, residing at San Francisco, in the county of San Francisco and State of California, have invented certain new and useful Improvements in the Concentration of Ores, of which the following is a specification.

This invention is for improvements in or relating to ore concentration and relates more particularly to the processes of the type generally known as the froth flotation processes.

The invention is in some respects a development from that covered in the United States Patent No. 962,678.

It has been found that there are a number of hydrocarbons, particularly unsaturated hydrocarbons, which when treated with sulfuric acid form compounds very suitable for use as frothing agents in the froth flotation processes of ore concentration and with some ores these agents have advantages in forming a cleaner concentrate or a more stable froth. These products are obtained in the treatment and refining of hydrocarbons, such as petroleum, kerosene, gas-tar and the like, and particularly in the refining of their distillates. A typical example of such products is known as acid sludge, and it has been found, for example, that acid sludge produced by the sulfuric acid treatment of kerosene obtained from California petroleum is highly advantageous as a frothing agent.

In the employment of the agitation froth process as described for example in the United States Patents Nos. 835,120 and 962,678, difficulties are frequently encountered when the ore pulp contains very fine gangue slimes or colloidal gangue slimes. This is frequently the case for example with copper ores and the use of the compounds produced by the action of sulfuric acid on hydrocarbons of the type described has proved especially advantageous in such cases. Excellent results have been obtained for example by using these frothing agents in the sub-aeration process of ore concentration as described for example in the United States Patents Nos. 1,155,836 and 1,155,815.

The following is an example of the operation of this process. The material operated was the tailings from water concentration tables in the treatment of copper ore from

the Anaconda mines, Montana, and these tailings assayed 2.26% of the copper. To a pulp containing this material in the proportion of 24.0% of solids, was added 2.3 lbs. acid sludge per ton of material treated, 2.3 lbs. wood creosote per ton of material treated, .21 lbs. stove oil per ton of material treated, 12.7 lbs. sulfuric acid per ton of ore. The pulp heated to 97° Fahrenheit was treated in a standard mineral separation flotation machine wherein it was agitated to form a froth and the froth was separated. The concentrates assayed 10.1% copper and the tailings assayed .2% copper. It is further found that these substances produced by the action of sulfuric acid on hydrocarbons are, in many cases, more effective as frothing agents when they have been standing for some time, or when they have been mixed with water for some time, and this invention includes the use of such compounds in these conditions.

This invention may be used in conjunction with any of the known or patented processes of ore concentration by froth flotation, either for the separation of the metalliferous constituents of an ore from the gangue, or for the separation of different metalliferous constituents from one another.

I claim:

1. A process of concentrating ores which consists in mixing the finely crushed ore with water, adding a minute quantity of a product obtained by treating a hydrocarbon (composed exclusively of hydrogen and carbon) with sulfuric acid, agitating and aerating the mixture to form a froth, and separating the froth.

2. A process of concentrating ores which consists in mixing the finely crushed ore with water, adding a minute quantity of a product obtained by treating a mixture of hydrocarbons (composed exclusively of hydrogen and carbon) with sulfuric acid, agitating and aerating the mixture to form a froth, and separating the froth.

3. A process of concentrating ores which consists in mixing the finely crushed ore with water, adding a minute quantity of a product obtained by treating a hydrocarbon (composed exclusively of hydrogen and carbon) with sulfuric acid, and a small quantity of acid, agitating and aerating the mixture to form a froth, and separating the froth.

851

80

95

105

110



acid sludge obtained by treating petroleum distillate with sulfuric acid, and a small quantity of sulfuric acid, agitating and aerating the mixture to form a froth, and separating the froth.

19. A process of concentrating ores which consists in mixing the finely crushed ore with water, adding a minute quantity of acid sludge obtained by treating petroleum distillate with sulfuric acid and allowing it

to stand for some time, and a small quantity of sulfuric acid, agitating and aerating the mixture to form a froth, and separating the froth.

In testimony whereof I have affixed my <sup>15</sup> signature in presence of two witnesses.

EDWARD HOIT NUTTER.

Witnesses:

JED SILVEY,  
CHESTER B. ALLEN.